

**UNITED STATES PATENT OFFICE**

2,129,414

# PROCESS FOR TREATING YARNS, FIBERS, AND FILAMENTS

Wendell G. Faw, Kingsport, Tenn., assignor to  
Eastman Kodak Company, Rochester, N. Y.,  
a corporation of New Jersey

**No Drawing. Application March 27, 1937,  
Serial No. 133,426**

9 Claims. (Cl. 28—1)

This invention relates to the conditioning of textile yarns and more particularly to the conditioning of filaments and yarns composed of organic derivatives of cellulose such as cellulose acetate, cellulose acetate propionate, cellulose acetate butyrate, etc., to render them more amenable to textile operations such as knitting and particularly for circular knitting.

and particularly for circular knitting.

As is well known, in the manufacture of yarns, particularly those composed of or containing cellulose organic derivatives, it is necessary to treat the yarn in order to reduce the tendency toward breakage of the individual filaments or fibers when they are subjected to various mechanical strains and to lubricate the yarn in order to facilitate handling in such operations as spinning, twisting winding and reeling. In addition, it is necessary to treat yarn to adapt it for use as warp or filling or for the manufacture of various types of knitted fabrics. In knitting, it is particularly important that the yarn be soft and pliable in order that it may conform readily to the contour of the needles and thus produce a closely knit fabric free from such defects as "stitch distortion", "pin holes", "laddering" and the like.

Heretofore it has been proposed to employ softening agents such as polyhydric alcohols and similar agents as ingredients of yarn conditioning or lubricating formulae, generally in connection with mineral, animal or vegetable oils. It has been found, however, that most of the known softening agents and the various formulae containing them have certain drawbacks, one of the most serious of which is high vapor pressure, and in some cases too drastic a solvent action on the yarn. Many of such agents possess slight or insufficient solvent power for the lubricants with which they are used and it is accordingly necessary to employ blending agents or emulsifying agents in order to obtain operable yarn treating formulae. In addition, many of the known softening and lubricating agents are insufficiently soluble in water to permit satisfactory removal by aqueous scour baths.

45 factory removal by aqueous soap baths.

This invention has as its principal object to provide an entirely new class of yarn conditioning agents which are particularly adapted for the treatment of yarns composed of or containing 50 organic derivatives of cellulose and capable of lubricating, softening and rendering such yarns more amenable to knitting and other textile operations. A further and specific object is to provide a class of conditioning agents which 55 augment or assist the lubricating action of vari-

ous lubricants when applied to such yarns. A still further object is to provide yarn softening and lubricating formulae which can be readily removed from the yarns by the usual scour baths. A still further object is to provide an improved method for the conditioning of yarns, particularly those composed of or containing organic derivatives of cellulose such as cellulose acetate, whereby the yarn is rendered soft and pliable and capable of employment in a variety of textile operations where complicated designs or stitches are employed. Other objects will appear hereinafter. 5 10

These objects are accomplished by the following invention which, in its broader aspects, comprises the discovery that beta-methoxy ethyl succinate, a diester of succinic acid having the following structure:



may be used as a yarn conditioning agent and particularly as a softening agent, with or without the addition of animal, mineral or vegetable oils, in the treatment of yarn composed of or containing organic derivatives of cellulose. 30

I have found that this compound has a slight solvent and/or softening action on cellulose organic derivative yarns which renders such yarns soft and pliable without at the same time having too drastic a solvent action thereon. 35

This compound also has a particular advantage over other solvents or yarn softening agents in that it has a very low rate of evaporation. Yarn treated with this compound will not lose its softness on exposure to the atmosphere over a comparatively long period of time. 40

In the following examples and description I have set forth several of the preferred embodiments of my invention, but they are included merely for purposes of illustration and not as a limitation thereof.

*Example 1.*—Yarn designed for knitting and composed of cellulose acetate is treated by applying thereto a composition having the following formula:

|                              | Parts by weight |
|------------------------------|-----------------|
| Beta-methoxy ethyl succinate | 85              |
| Oxidized olive oil           | 15              |

The amount of the conditioning liquid may run 55

anywhere from 1-25% of the weight of the yarn, 5-25% being the preferable amount.

*Example II.*—The cellulose acetate 150 denier yarn is treated by applying thereto by means of an applicator roll as the yarn emerges from the spinning cabinet 5-25%, based on the weight of the yarn, of a composition having the following ingredients:

| Parts by weight |                              |    |
|-----------------|------------------------------|----|
| 10              | Beta-methoxy ethyl succinate | 70 |
| 15              | Fatty alcohol                | 20 |
| 20              | White mineral oils           | 10 |

*Example III.*—A yarn conditioning liquid is made up by mixing the following ingredients in the indicated proportions:

| Parts by weight |                              |    |
|-----------------|------------------------------|----|
| 10              | Beta-methoxy ethyl succinate | 30 |
| 15              | Diamyl tartrate              | 10 |
| 20              | Oxidized sperm oil           | 10 |

This composition is applied to 100 denier cellulose acetate yarn intended for knitting in an amount representing 5-25% by weight of the yarn. The filaments or fibers of the yarn treated as described above are quite soft and pliable and give excellent results in textile operations, especially knitting.

As will be apparent from the above examples and description, the conditioning agents of my invention may be applied by a wide variety of methods. For example, we may employ the agent as an ingredient of the spinning dope from which the filaments are formed, the amount of the agent so employed depending upon a number of factors such as the particular cellulose derivative used in making the yarn, the solvent or solvent combination used in making up the spinning solution, and the degree of softness or pliability desired in the yarn, etc.

If the conditioning agent is to be applied to the yarn after spinning, this may be done by bringing the yarn in contact with a wick, roll, or felt wet therewith, or the liquid may be applied by immersion, spray, or otherwise. The particular point at which the liquid is applied may vary. It may, for example, be applied to the yarn inside or outside the spinning cabinet, between the guide and godet roll, between the godet or other roll or guide and the point of winding and/or twisting. In some cases, the liquid may even be applied to the yarn after winding onto cones, spools, bobbins, or the like or by the so-called "bobbin to bobbin" method. In the case of staple fiber manufacture, the liquid may be applied to the yarn prior to, or after cutting into staple lengths.

The amount of the agent so employed will vary widely depending upon the results desired, the specific nature of the material to which the agent is applied, the use to which the yarn is eventually to be put and other factors. For example, in a given case where a cellulose organic acid ester yarn such as a yarn composed of cellulose acetate, is intended for circular knitting, about 10-15% or more by weight, based on the weight of the dry yarn, may be satisfactory, while if the yarn is intended for weaving, the amount may vary between about 2 and 5%.

There is also a slight difference in the requirements of dull luster as compared to bright luster yarn with respect to the amount of conditioning agent applied. In general, it may be said that when a dull luster yarn, for example, yarn produced from a cellulose acetate spinning solution and containing a delustering agent such as finely

divided titanium oxide, is conditioned by my method, I prefer to use 5%-15% of the conditioning agent. With bright luster yarn, that is, yarn produced from a clear spinning solution containing no delustering agent, I prefer to use 5 1%-5% of the conditioning agent.

Although in the above examples I have referred primarily to yarn treating compositions containing only the conditioning agent and an oil, other ingredients such as solvents, non-solvents, emulsifying agents, blending agents and the like, may be added within the scope of my invention. In fact, any other component that will be miscible with the mixture of oil and beta-methoxy ethyl succinate may be added. I have found, for example, that dibutyl phthalate, diamyl tartrate, fatty alcohols, such as lauryl, oleyl, etc., and other plasticizing or similar agents may be added. Likewise, various dyes or other coloring matter may be included in case it is desired to permanently or fugitively tint or dye the material undergoing treatment.

Although I have found it convenient to illustrate my invention by reference to compositions containing specific percentages of the various ingredients, these percentages may vary widely depending upon the particular purpose for which the composition is intended. For example, if it is desired to control the solvent or softening action of the conditioning agent, the amount of the agent may be adjusted as, for example, by reducing the amount of the agent and correspondingly increasing the amount of oil or other ingredient.

While I have described my invention with particular reference to the treatment of yarns composed of organic derivatives of cellulose such as cellulose acetate, the conditioning agents and formulae described herein are applicable to the conditioning of many other types of cellulose derivative yarns such as those composed of or containing cellulose propionate, cellulose butyrate, cellulose acetate propionate, cellulose acetate butyrate, ethyl cellulose, methyl cellulose, benzyl cellulose and others.

The term "yarn" as used herein and in the claims is to be understood as including a single filament, a plurality of filaments associated into the form of a thread, either of high or low twist, single or multiple threads associated or twisted together, composite threads composed of a mixture of natural and artificial filaments or a composite thread formed by twisting together individual strands of natural or artificial materials, as well as cut staple fibers produced from natural and/or artificial filaments or threads and spun yarn produced from such staple fibers.

As indicated above, the yarn conditioning agents of my invention are exceptionally good solvents for a wide variety of mineral, blown and unblown, drying and semi-drying animal and vegetable oils such as cottonseed, olive, castor, neat's-foot, sperm and other oils. This enables them to be used with any of such oils in making up a variety of yarn treating formulae of varying composition.

The yarn conditioning method and compositions of my invention possess many outstanding advantages. The fundamental and outstanding characteristic of the agents employed in accordance with the invention is their ability to soften yarns, especially those composed of or containing organic derivatives of cellulose such as cellulose acetate and render them soft and pliable and amenable to various textile operations, especially

operations such as those involved in weaving and knitting where complicated designs or stitches are employed, without too drastic an action on the yarn material. Another outstanding characteristic of this compound is its exceptional solvent power for a wide variety of mineral, animal and vegetable oils and its ability to act as lubricating assistant in conjunction with these oils when applied to such yarns. In addition, due to its solubility in water, it may readily be removed from yarns and fabrics by means of the usual aqueous scour baths. By employing the yarn conditioning agents and methods of our invention as herein described, one is enabled to obtain highly satisfactory results in the manufacture of yarns and woven fabrics and especially the production from these yarns of knit fabrics free from defects such as pin holes, stitch distortion, laddering and the like.

20 What I claim and desire to secure by Letters Patent of the United States is:

1. The process of conditioning yarn to render it more amenable to textile operations including circular knitting, weaving, spinning and the like which comprises applying thereto a lubricating and softening composition containing beta-methoxy ethyl succinate.

2. The process of conditioning yarn composed of or containing organic derivatives of cellulose to render it more amenable to textile operations including circular knitting, weaving, spinning and the like which comprises applying thereto a lubricating and softening composition containing meta-methoxy ethyl succinate.

35 3. The process of conditioning yarn composed of or containing cellulose acetate to render it more amenable to textile operations including circular knitting, weaving, spinning and the like, which comprises applying thereto a lubricating

and softening composition containing beta-methoxy ethyl succinate.

4. The process of conditioning yarn composed of or containing cellulose acetate to render it more amenable to textile operations including 5 circular knitting, weaving, spinning and the like, which comprises applying thereto a lubricating and softening composition containing beta-methoxy ethyl succinate and a textile lubricant.

5. Textile yarn amenable to textile operations 10 including circular knitting, weaving, spinning and the like, impregnated with a lubricant containing beta-methoxy ethyl succinate.

6. Textile yarn composed of or containing organic derivatives of cellulose amenable to textile 15 operations including circular knitting, weaving, spinning and the like, impregnated with a conditioning agent comprising beta-methoxy ethyl succinate.

7. Textile yarns composed of or containing 20 cellulose acetate amenable to textile operations including circular knitting, weaving, spinning and the like, impregnated with a lubricating and softening composition containing beta-methoxy ethyl succinate.

25 8. A conditioning agent for rendering yarns more amenable to textile operations including weaving, spinning, knitting and the like which is composed of 70-80 parts by weight of beta-methoxy ethyl succinate, the balance being a 30 textile lubricant.

9. A conditioning agent for rendering yarns more amenable to knitting having the following formula:

|                              | Parts by weight | 35 |
|------------------------------|-----------------|----|
| Beta-methoxy ethyl succinate | 85              |    |
| Oxidized olive oil           | 15              |    |

WENDELL G. FAW.